

# UNITED STATES PATENT OFFICE.

BERTHOLD GUSTAV RESCHKE, OF HAMBURG, GERMANY.

## SAFETY-EXPLOSIVE.

No. 882,910.

Specification of Letters Patent. Patented March 24, 1908.

Application filed June 19, 1906. Serial No. 323,447.

To all whom it may concern:

Be it known that I, BERTHOLD GUSTAV RESCHKE, a citizen of the German Empire, and resident of Hamburg, Germany, have invented a new and improved Safety-Explosive, of which the following is a specification.

This invention relates to safety explosives more particularly for use in mines where it is most important to consider the effects of the explosion gases, and its object is to provide safety explosives that shall generate explosion gases of a harmless nature and more highly advantageous than is the case with existing explosives. For this purpose the seeds of fennel, (*Foeniculum*), either ground or unground, are mixed with ammonium nitrate, or both said ingredients may be jointly ground in a suitable mill. To the above mixture other substances may be added, as hereinafter described.

The following are examples of the composition of my safety explosives:

|    |                        |
|----|------------------------|
| 25 | 86.0% ammonium nitrate |
|    | 14% fennel             |
| or | 85.5% ammonium nitrate |
|    | 1.0% dinitrobenzol     |
|    | 13.5% fennel           |
| 30 | 94.0% ammonium nitrate |
|    | 6.0% fennel            |
| or | 95.0% ammonium nitrate |
| 35 | 1.0% dinitrobenzol     |
|    | 4.0% fennel            |

These safety explosives have great power and are not readily affected by lengthy storing. This great explosive power is due to the 40 large percentage of ethereal oils contained in the seeds of fennel. However, I have ascertained that the explosive energy and the resulting explosion gases can be greatly improved by the admixture of fine wood pulp 45 to the aforementioned explosives, thus:—

|    |                        |
|----|------------------------|
| 50 | 87.0% ammonium nitrate |
|    | 7.0% fennel            |
|    | 6.0% wood pulp         |
| or | 86.7% ammonium nitrate |
|    | 1.0% dinitrobenzol     |
|    | 6.6% fennel            |
|    | 5.7% wood pulp         |

|                                                                                                                                                                                                                                          |    |
|------------------------------------------------------------------------------------------------------------------------------------------------------------------------------------------------------------------------------------------|----|
| 94.3% ammonium nitrate                                                                                                                                                                                                                   | 55 |
| 3.0% fennel                                                                                                                                                                                                                              |    |
| 2.7% wood pulp                                                                                                                                                                                                                           |    |
| or                                                                                                                                                                                                                                       |    |
| 95.2% ammonium nitrate                                                                                                                                                                                                                   | 60 |
| 1.0% dinitrobenzol                                                                                                                                                                                                                       |    |
| 2.0% fennel                                                                                                                                                                                                                              |    |
| 1.8% wood pulp                                                                                                                                                                                                                           |    |
| The addition of wood pulp is of great advantage in the manufacture of these explosives, as it absorbs the oils contained in the fennel seeds, so that any sticking of the mixture to the reducing mill or mixing apparatus is prevented. | 65 |
| In order to render the same practically safe from fire-damp explosions I use the following constituents and proportions viz:                                                                                                             | 70 |
| 81.5% ammonium nitrate                                                                                                                                                                                                                   |    |
| 13.5% fennel                                                                                                                                                                                                                             |    |
| 5.0% copper-oxalate                                                                                                                                                                                                                      | 75 |
| or                                                                                                                                                                                                                                       |    |
| 81.8% ammonium nitrate                                                                                                                                                                                                                   |    |
| 6.6% fennel                                                                                                                                                                                                                              |    |
| 5.6% wood pulp                                                                                                                                                                                                                           |    |
| 1.0% dinitrobenzol                                                                                                                                                                                                                       | 80 |
| 5.0% copper-oxalate                                                                                                                                                                                                                      |    |
| 69.6% nitrate of ammonia                                                                                                                                                                                                                 |    |
| 10.0% nitrate of potash                                                                                                                                                                                                                  |    |
| 14.4% fennel                                                                                                                                                                                                                             |    |
| 1.0% dinitrobenzol                                                                                                                                                                                                                       | 85 |
| 5.0% oxalate of copper                                                                                                                                                                                                                   |    |
| or                                                                                                                                                                                                                                       |    |
| 70.4% nitrate of ammonia                                                                                                                                                                                                                 |    |
| 10.0% nitrate of potash                                                                                                                                                                                                                  |    |
| 7.2% fennel                                                                                                                                                                                                                              |    |
| 6.4% wood-pulp                                                                                                                                                                                                                           |    |
| 1.0% dinitrobenzol                                                                                                                                                                                                                       |    |
| 5.0% oxalate of copper                                                                                                                                                                                                                   | 90 |

What I claim is:

1. An ammonium nitrate explosive consisting of ammonium nitrate and fennel seed, in about the proportions stated.
2. An ammonium nitrate explosive consisting of ammonium nitrate, fennel seed and wood pulp, in about the proportions stated.

Signed at Hamburg this 5th day of June 1906 in presence of two witnesses.

BERTHOLD GUSTAV RESCHKE.

Witnesses:

FRIEDRICH I. POTHO,  
OTTO W. HELLMRICH.